# EUROPEAN PATENT SPECIFICATION

(11) **EP 0 059 296 B1**
(45) Date of publication and mention of the grant of the patent: **02.05.1984**
(21) Application number: 81830137.6
(22) Date of filing: 29.07.1981
(51) Int. Cl.: C10M 3/22, C10M 1/28, B21D 39/20

(54) **Application of polyglycols soluble in water as lubricant in mechanical expanders effecting the cold straightening and gauging of lengthwise welded steel tubes**
Verwendung von wasserlöslichen Polyglykolen als Schmiermittel in mechanischen Expandern für das Kaltrichten und Kalibrieren von Langsnahtstahlrohren
Application de polyglycols solubles dans l'eau comme lubrifiants dans des dispositifs à expansion mécanique de tubes en acier à joint soudé longitudinalement effectuant le redressage à froid et le calibrage

(43) Date of publication of application: 08.09.1982
(73) Proprietor: VISCOSUD of Dott.Ing. Mario Fiorese S.r.l., Bari (IT)
(72) Inventor: Fiorese, Mario, Dott. Ing., Bari (IT)
(74) Representative: Russo, Saverio, Dott. Ing.

## Description

The invention refers to a new application of polyglycols soluble in water, with high EP - extreme pressure - properties, to lubricate heavy operating machines in which sliding frictions take place at a high pressure due to the reciprocal sliding of the surfaces of the working members: more in detail, it is concerned with a new application of polyglycols obtained by copolymerisation of ethylene oxide and propylene oxide as lubricants to waste after each working cycle, in machines in which the operating conditions are identical to the ones that take place in a mechanical expander made by Mannesmann Meer AG Mönchengladbach, better known as a cold doublehead mechanical expander with two expansion units. A. O. Smith system, to effect the straightening of tubes with a diameter from 0,76 to 1,42 m (30 to 56 inches), thick from 6,35 to 25,4 mm, length from 10 to 18 m ± 200 mm, in order to correct the "banana" effect due to the welding and to carry out their gauging.

This machine (see figure), that has been preferred to the expanders of hydraulic type because of its better functioning, is formed by a truncated pyramid or wedge 1 and by wedge-shaped elements 2 placed side by side and joined together by means of a ring so to form with their outer surface a cylindrical surface.

The wedge-shaped elements 2 slide simultaneously on the surface of the wedge 1, and move radially in a centrifugal direction, conveying their pressure on the inner surface of a tube 4 if a tension-rod 3 moves in the direction of the arrow.

So each expander needs a lubricant qualified to absorb the high pressures that can exceed 12 kg/sq.mm, because of the friction that takes place between the surfaces of the wedge-shaped element 2 and of the wedge 1 that causes the expansion, which are in reciprocal contact.

Moreover as the lubricant falls in the tube, it is almost always necessary to clean the inner surface of the tube at the end of the straightening, if the conditions of the inner surface of the tube must be checked visually and if other treatments such as sandblasting and special varnishings must be carried out.

At present, the builder of these expanders suggests using as lubricant EP - extreme pressure -, mineral oils that are emulsifiable in water; consequently in order to remove the lubricant that wets the inner surface of the tube, at the end of the every working cycle, chemical solvents must be used.

As the solvents are polluting and not biodegradable products and the lubricant contains slags and ferrous scales due to the cold-working of the expander, and the lubricant itself is a polluting substance, it is preferable to discard them rather than to recover them.

On the other hand, the discharge of the lubricant into water would give rise to further considerable expenses and to a considerable increase in the cost of the finished tubes, it being necessary to carry out treatment of great quantities of exhausted lubricant to avoid pollution, before discharging it. The mechanical expander above mentioned, built by Mannesmann, produces daily hundreds Kilos of waste lubricant.

From FR-A-2 299 472 it is known to use watersoluble polyglycols alone or in combination with oleic acid as lubricant in metal working operation.

It is also known from FR-A=2 243 035 to use water-soluble lubricants in mechanical expander processes.

The invention as claimed is intended to remedy these drawbacks due to the of emulsifiable EP lubricating oil in this type of expander for welded tubes and in other operating machines in which the same lubricating conditions take place i.e. soiling the worked surfaces by the lubricant and wasting of the exhausted lubricant itself.

The invention provides the use of a water soluble lubricant comprising an ethylene oxide propylene oxide copolymere having a load carrying capacity of _{>} 12 kg/mm² and suitable to consent the selectively removing of slags and ferrous scales that have settled on the lubricant wetting the wedge of the expander by washing with water at a pressure below 4 kg/cm² and subsequently removing the lubricant from the inner surface of the tube by washing at a pressure above 4 kg/cm².

The applications as lubricant of the polyglycols obtained by copolymerisation of ethylene oxide and propylene oxide soluble in water, with high EP properties (resistance to specified pressures greater than 12 kg./sq.mm) and high viscosity solves the general problem connected with a reduction of manufacturing costs of the welded tubes, because of the lower cost of such lubricant compared with the cost of the mineral lubricating oils and because of the possibility of discharging directly the exhausted lubricant into water without submitting it to particular treatments if its concentration is within the allowed limits.

Furthermore, the use of such polyglycols enables entire removal of the lubricant that falls into the tube or removal of just the slag and the ferrous scale that have settled on the lubricant wetting the wedge of the expander, by washing the tube and the wedges, without using a chemical substance, but only using water at different pressures: higher pressure to clean the tube and lower pressures removing only the slag and ferrous scale from the wedges.

In fact, the above mentioned polyglycols remain adherent to the lubricated surfaces of the machine if it undergoes a low pressure water washing (for instance 3-4 kg/sq.cm), whereas it is remove if it undergoes high pressure water washing.

These properties can be attained by means of copolymerisation of propylene oxide (C₃H₆0) and of ethylene oxide (C₂H₄0) to which are added vegetable oils and derivatives in percentages not higher than 10%.

When using the above mentioned Mannesmann cold mechanical double-head expander, with the above mentioned copolymeres as lubricants, if sandblasting and varnishing are required, the following final operations are needed:
a) cleaning of the inner surfaces of the tubes, wetted by the lubricant and of the working member of the expander by washing them with water at different pressures;
b) visual quality testing;
c) sandblasting and varnishing;
d) direct discharge of the exhausted lubricant in the drain water tanks of the factory because of its solubility and its lower toxicity. The use of the polyglycols owing to the fact that they can be discharged in great quantities in water, due to their lower toxicity also achieves extra advantages for the industries concerned with this problem because it allows simplification of the equipment and the plants meant for the treatment of industrial waste.

This would not be possible when mineral lubricating oils are used because of the extremely low concentration of said lubricating oil allowed in the drain water tanks of the factory (in Italy for instance the allowed concentration is 3 p.p. million).

## Claims

Use of a water soluble lubricant in the process of cold straightening and gauging of lengthwise welded steel tubes in a mechanical expander, to lubricate the surface between the central wedge (1) and the external wedge shaped elements (2) sliding on said wedge and moving radially in a centrifugal direction as the result of the motion of a tension rod (3), characterized by
(a) a lubricant comprising an ethylene oxide propylene oxide copolymer having a load carrying capacity of > 12 kg/mm²;
(b) selectively removing slags and ferrous scales that have settled on the lubricant wetting the wedge of the expander by washing with water at a pressure below 4 kg/cm², and
(c) subsequently removing the lubricant settled on the inner surface of the tube by washing with water at a pressure above 4 kg/cm².

## Patentansprüche

Verwendung eines wasserlöslichen Schmiermittels in mechanischen Expandern zum Kaltrichten und Kalibrieren von Langsnahtstahlrohren, zur Schmierung der gegenüberliegenden Aussenflächen des Zentralkeils 1 under der, auf diesem Keil, gleitenden und sich, infolge der Bewegung einer Zugstange 3, in zentrifugalradialer Richtung fortbewegenden Aussenkeilstucken 2, dadurch gekennzeichnet dass:
a) das Schmiermittel ein Äthylen-Oxyd Propylen-Oxyd Copolymer mit einer Belastbarkeit von mehr als 12 Kg/mm², enthält;
b) bei einem Wasserdruck von weniger als 4 Kg/cm², nicht das Schmiermittel von der Aussenfläche des Zentralkeils 1 entfernt wird, sondern die das Schmiermittel verunreinigenden Eisenschlacken und Eisenschuppen;
c) das Schmiermittel bei einem Wasserdruck von mehr als 4 Kg/cm², von der Rohrinnenwand entfernbar ist.

## Revendications

Utilisation d'un lubrifiant soluble dans l'eau, dans le procédé de rectification et calibrage à froid des tubes en acier soudés selon leur longueur, lequel fait usage d'un expanseur mécanique, pour lubrifier la surface de glissement entre le coin central 1 et les éléménts en forme de coin 2 lesquels, glissant sur ledit coin central 1, se deplacent radialement dans une direction centrifuge à cause du mouvement d'une tige de tension 3, ladite utilisation étant caracterisée par le fait que:
a) ledit lubrifiant soluble dans l'eau comprend un copolymère de l'oxyde d'éthylène et de l'oxyde de propylène et il est en mesure de supporter une charge de travail supérieure à 12 Kg/ₘₘ₂;
b) les scories, les crasses et les écailles de fer, ayant été introduites dans ledit lubrifiant lorsque celuici lubrifie le coin de l'expanseur, sont enlevéés sélectivement du lubrifiant, moyennant un lavage à l'eau sous une pression inférieure à 4 Kg/cm²;
c) ledit lubrifiant, deposé sur la surface interne desdits tubes, est enlevé successivement, moyennant un lavage a l'eau sous une pression supérieure à 4Kg/cm².
